

# UNITED STATES PATENT OFFICE.

FRED K. BEZZENBERGER AND MALCOLM N. RICH, OF CLEVELAND, OHIO, ASSIGNEES  
TO THE ALUMINUM CASTINGS COMPANY, OF CLEVELAND, OHIO, A CORPORATION  
OF OHIO.

## CASTING AND PROCESS OF TREATING CASTINGS AND THE LIKE.

1,383,517.

Specification of Letters Patent.

Patented July 5, 1921.

No Drawing.

Application filed November 24, 1919. Serial No. 340,406.

To all whom it may concern:

Be it known that we, FRED K. BEZZENBERGER and MALCOLM N. RICH, citizens of the United States, residing at Cleveland, in the county of Cuyahoga and State of Ohio, have invented certain new and useful Improvements in Casting and Processes of Treating Castings and the like, of which the following is a specification, reference being had therein to the accompanying drawing.

This invention relates to the treatment of metallic articles whereby pores or small openings therein are substantially stopped and the articles thereby rendered impervious to fluids. The treatment is applicable to all metallic articles which are porous, but is of special importance with castings of alloys of aluminum and other light metals which are subject to relatively great porosity and which should for many purposes be impenetrable by air, water, gasoline and other fluids.

One object of the invention is to provide an improved method of rendering porous metallic articles substantially impervious to fluids.

Another object is to provide a method for the treatment of porous metallic articles by which a relatively inert material is formed within the pores of such articles whereby the said pores are stopped and the passage of fluids through the said articles prevented.

Another object is to devise a method or process for the treatment of porous metallic articles according to which anhydrous silica may be formed within the pores of the porous articles.

Another object is to provide a method of treatment for porous metallic articles by which a relatively inert or insoluble material is formed independently of the metals comprising the said articles.

Another object is to produce a metallic article, the pores of which are stopped with relatively inert or insoluble material.

Other objects will appear to those skilled in the art from the following description of the method and the preferred means of practising it.

Our process consists briefly in the formation, by chemical reactions within the pores of the articles, of solid precipitates practically insoluble in water or other common

solvents. It is applicable to any metallic article which is relatively porous, because it is not dependent on the metal or metals comprising the article, provided however that the solutions which are employed, do not react harmfully on the articles to be treated. Since the process is especially valuable in the treatment of aluminum alloy castings, the method will for purposes of illustration, be described as carried out with such castings.

In the casting of aluminum alloys, especially in sand molds, difficulty has been experienced in making the castings sufficiently non-porous to prevent passage therethrough of such fluids as air, water, gasoline, etc. These fluids, in fact, are commonly used to test the porosity of aluminum alloy castings, some fluids frequently being applied under a pressure of several pounds per square inch, although ordinarily no pressure is applied.

According to the preferred method of practising our invention castings which have been found to leak when subjected to air, water, or other fluids, are treated as follows: The casting is first immersed in a bath of concentrated sodium silicate for about an hour, then the casting is removed and dipped for one or two minutes in a bath of dilute sulfuric acid. Following this dipping, the casting is rinsed with water and then heated at a temperature of 100° C. (212° F.) for an hour or more.

It is obvious that a solution of any soluble silicate may be used but for purposes of illustration, we have selected sodium silicate as being preferable. While baths of varying degrees of concentration may be employed, a concentrated bath of sodium silicate (40° Baumé; 1.38 specific gravity) has given good results.

It has been found in practice that a concentrated solution tends to retard the process where the pores in the article being treated are relatively small, and that, on the other hand, dilute solutions do not always produce, in a single treatment, a stoppage of the pores. This is due to the fact that a concentrated solution of sodium silicate is rather viscous and does not readily enter small openings in the articles being treated, while the dilute solutions do not contain sufficient sodium silicate to produce, after

precipitation, a quantity of silica which will stop the pores.

To insure penetration of the solution into the many small openings in the casting, it is desirable to immerse the casting in the silicate solution, the duration of the immersion depending on the size and thickness of the casting, the sizes of the openings or pores therein and the degree of concentration of the silicate solution. If the casting is very porous the solution will readily enter the pores but if the openings are small, a longer soaking is necessary to insure penetration to all the interstices. The length of time the articles should be immersed may, therefore, vary widely under different conditions, the period of about an hour specified in our preferred method having been found to give satisfactory results with the common aluminum alloys constituting articles such as automobile engine crank case and smaller parts cast in sand molds.

Several different acids might be used and in varying strengths with good results but we prefer to use a mineral acid such as hydrochloric acid, sulfuric acid or acid sodium sulfate. Baths of hydrochloric or sulfuric acid which have been found suitable were made by mixing one part of concentrated commercial grade acid with six parts of water. A suitable bath of acid sodium sulfate may be made by adding ten parts by weight of the sulfate to 100 parts by weight of water.

The action of the acid bath is to cause a precipitation of hydrosilicic acid or hydrous silica within the pores or openings of the casting as well as on the surfaces thereof, according to the chemical reaction.



Subsequent washing with water removes the silica, soluble salts and excess acid from the surfaces of the casting leaving within the pores of the casting, the hydrous silica formed therein. The hydrosilicic acid or hydrous silica is freed from part of its uncombined water and is partly converted into its less soluble form, anhydrous silica, by the application of heat to the castings, some of the hydrous silica being decomposed with the formation of water and anhydrous silica. Ordinarily heating the casting for an hour at a temperature above the boiling point of water will give satisfactory results but they may be heated at a lower temperature for longer periods if desired. The pores are thus substantially stopped with the insoluble silica and leakage through the casting is prevented. Repeated treatments may be made if necessary, where, as in the case of the castings having relatively large pores, the pores are not completely closed with the first treatment.

The final step of applying heat to the

treated articles might be dispensed with but we prefer not to omit it because the hydrous silica is more easily soluble than the anhydrous form, and might, therefore, be dissolved and washed out of the pores of the casting. Furthermore, the anhydrous silica has no tendency to drain out of the pores as might be the case if the excess water and acid were not removed from the pores of the casting by volatilization.

75

While we have set forth for purposes of illustration, a particular and preferred method of practising the invention, it is to be understood that the method is not limited to the exact steps described but is limited only by what is claimed in the appended claims.

What we claim is:

1. The method of rendering porous metallic articles impervious to fluids which comprises the formation of silica within the pores of the said article and the partial dehydration of the silica.

2. The method of rendering porous metallic articles impervious to fluids, which comprises, first causing a solution of a silicate to enter the pores in the article; second, bringing an acid solution into contact with the silicate solution within the said pores; and third, heating the said article.

95

3. The method of rendering porous metallic articles impervious to fluids which comprises immersing the article in a bath of sodium silicate; then dipping the article in a bath of mineral acid; washing the surface of the casting with water; and finally heating the article.

100

4. The method of rendering porous metallic articles impervious to fluids such as air, water or gasoline, which consists in, first, immersing the article in a bath containing a soluble silicate; second, dipping the article in a bath containing an acid capable of reacting chemically with the soluble silicate to precipitate hydrosilicic acid; third, rinsing excess materials from the surfaces of the article; and fourth, heating the article to convert a part of the hydrosilicic acid into anhydrous silica.

105

5. The method of rendering porous metallic articles impervious to fluids such as air, water or gasoline which consists in, first immersing the article in a bath containing sodium silicate until the solution has penetrated the pores of the said article; second, dipping the article in a bath containing sulfuric acid whereby hydrosilicic acid is precipitated within the pores of the article; third, washing excess materials from the third, washing excess materials from the surfaces of the article, and fourth, heating the within the pores of the article is converted into anhydrous silica.

110

6. The method of stopping the pores of aluminum alloy castings which consists in

125

130

- immersing the casting in a fluid reagent and causing the latter to penetrate the pores of the casting, subsequently immersing the casting in another fluid reagent which enters the pores and reacts with the first fluid contained therein to form a precipitate which stops the pores, and heating the casting to change the nature of the said precipitate.
5. As a new article of manufacture, a metallic article the pores of which are stopped with silica.
8. As a new article of manufacture, an aluminum alloy casting having its pores stopped with partially dehydrated silica.
- In testimony whereof we hereunto affix 15 our signatures.

FRED K. BEZZENBERGER.  
MALCOLM N. RICH.